

Sept. 16, 1941.

J. D. SEAVER

2,256,218

METHOD AND APPARATUS FOR CASTING PERMANENT MAGNETS

Filed Oct. 4, 1939

Fig.1.



Fig. 3.



Fig. 2.



Fig. 4.



Fig. 5.



Fig. 6.



Inventor:  
John D. Seaver,  
by Harry E. Dunham  
His Attorney.

## UNITED STATES PATENT OFFICE

2,256,218

METHOD AND APPARATUS FOR CASTING  
PERMANENT MAGNETS

John D. Seaver, Cohasset, Mass., assignor to General Electric Company, a corporation of New York

Application October 4, 1939, Serial No. 297,910

5 Claims. (Cl. 22—203)

The present invention relates to a method for casting permanent magnets and particularly to a method for casting magnets which are adapted for use in watt hour meters and like devices.

It is one of the objects of the present invention to provide a method and apparatus for simultaneously casting a plurality of pieces of permanent magnet alloys onto a metal base plate. A further object of the invention is to provide a method for casting economically small permanent magnets. Other objects will appear hereinafter.

The novel features which are characteristic of my invention are set forth with particularity in the appended claims. My invention itself however will best be understood from reference to the following specification when considered in connection with the accompanying drawing in which Fig. 1 is a plan view of a multiple mold and rotating casing therefor; Fig. 2 is a cross sectional view of the mold and casing illustrated in Fig. 1 when tilted to receive molten metal; Fig. 3 is a perspective view of one of the sand molds illustrated in Fig. 1 and a base plate for closing the openings in the mold and onto which the magnetic material is cast; Fig. 4 is a cross sectional view of the assembled sand mold and closure plate; Fig. 5 is a perspective view of a casting as removed from a mold; while Fig. 6 is a view in elevation of a trimmed casting and base plate as assembled in a meter yoke or shield.

In carrying out my invention I employ a permanent magnet alloy composition which has a very high coercive force, for example a magnet alloy of the well known alnico type which may consist of iron, nickel and aluminum or these elements in combination with others, for example cobalt, copper, titanium etc. The alloy preferably is a cast alloy and in fabricating it I employ a sand mold which, if desired, may consist of a plurality of similar molds as indicated at 1 on the drawing. Each mold has an upper opening 2 and a lower opening 3 which corresponds to the shape of the magnet polepieces 4 and 5 to be cast therein. In the fabrication of permanent magnets suitable for use in watt hour meters and the like, it may be desirable to employ a soft iron base plate 6 which serves to support polepieces 4 and 5 and also to form a continuation of the steel yoke or shield 7. If desired however the base plate 6 may be formed of any suitable material for example chrome steel or even non-magnetic metal. To secure a firm connection between the individual polepieces of the base plate, the latter is provided with projections 8 which are punched out of the iron as

indicated at 9. The upper ends of the projections 8 are slightly mushroomed, as indicated at 10.

In the casting operation the sand molds 1 are circumferentially arranged in a container 11 which is provided with an elevated platform 12 which supports the forward ends of the various molds 1 as indicated in Fig. 2. The container 11 is driven from a source of power, not shown, through a shaft 13 and it may be tilted from a horizontal position as indicated in Fig. 2. The container 11 is rotated at a desired speed and the metal alloy poured into the various openings 2 and 3 of the molds. The rotation of the molds forces the molten metal against the base plate 6 and around projections 8 so that polepieces 4 and 5 when cooled, are firmly attached thereto. When the necessary amount of molten metal has been poured into the molds and the metal has solidified to the desired extent the castings may be removed and the sprues 14 cut off and the upper surface of each polepiece ground to the desired extent after which it may be mounted in a meter structure or yoke 7 as indicated in Fig. 6.

My improved casting process and apparatus is particularly well adapted for the production of small permanent castings of the alnico type. Such castings may be made by my process with very short sprues which results in certain economies since the sprues are short enough to permit re-melting. If the castings were made with long sprues re-melting of such sprues might not be satisfactory because of difficulty in controlling the aluminum content of the resulting alloy. The grain structure of the resulting alnico type castings is very fine due to the churning and violent turbulence of the metal as it fills the molds and solidifies.

The fine grain results in an alloy of considerable strength which may be ground far more easily than castings made by the usual gravity process. Although fine grain castings may be obtained in a limited way by pouring gravity castings close to the freezing temperature of the metal, in my improved process for making permanent magnets of the alnico type close control of pouring temperature is not necessary since the metal may be poured at a higher temperature than that employed for making gravity castings.

The cast metal may be cooled in the mold if desired and at a rate which will effect a condition of precipitation and the desired magnetic characteristics in the alloy. If desired, however,

the alloy may be reheated at a temperature below the melting point to assure complete precipitation. Although I have illustrated my invention with a plurality of sand molds 1, it is obvious that a single multiple cavity mold could be employed if desired.

What I claim as new and desire to secure by Letters Patent of the United States, is:

1. A process for casting permanent magnet alloys which comprises rotating a mold having openings therethrough and a metal closure plate for the outer ends of said openings, and pouring molten metal into said rotating mold and onto said plate to thereby simultaneously form a pair of polepieces mounted on said plate.

2. A process for casting permanent magnet alloys which comprises rotating a mold having openings therethrough and a metal plate closing the outer ends of said openings, said plate having a projection thereon, pouring molten metal into said mold and around said projection to thereby simultaneously form a pair of polepieces mounted on said plate.

3. A mold having a plurality of openings therethrough and a metal plate closing said openings and onto which molten metal may be poured.

4. A mold having an upper and a lower opening extending therethrough and a metal plate closing said openings, said plate having a plurality of projections thereon extending into said openings and onto which the molten metal may be poured.

5. A centrifugal casting machine which comprises a supporting member, a multiple cavity mold arranged on said member, said mold having a plurality of pairs of circumferentially arranged openings extending therethrough, each pair of openings comprising an upper and a lower opening, a plurality of spaced metal plates, each plate closing the outer ends of a pair of said openings, means for rotating said supporting member, and means whereby molten metal may be poured directly into the openings in said mold and onto said closure plates.

JOHN D. SEAVER.